

Sept. 19, 1961

H. S. USEL

3,000,996

ACCUMULATORS

Filed June 27, 1957



Fluid - and Gas - Tight  
Accumulator containing:

Electrolyte,  
Electrodes,  
Absorbing Substances  
and  
Redox System Formers.

INVENTOR  
HUBERT STEPHAN USEL

BY Wenderoth, Lind & Bonack

ATTORNEYS

# United States Patent Office

3,000,996

Patented Sept. 19, 1961

1

3,600,996

## ACCUMULATORS

Hubert Stephan Usel, Sistrans (Tyrol), Austria  
Filed June 27, 1957, Ser. No. 668,505  
Claims priority, application Austria July 2, 1956  
6 Claims. (Cl. 136—9)

This invention relates to a fluid and gas-tight totally-enclosed accumulator.

In accumulators of such kind the formation of gases which may occur by loading, discharge, self-discharge and chiefly by overloading either has to be prevented or the gases must be bound. For example, in overloaded lead accumulators oxygen forms itself at the anode and hydrogen at the cathode.

Object of the invention is to prevent the formation of small gas-bubbles or to bind the occurring gases in the electrolyte, respectively in or at the electrodes.

A special purpose of this invention is to prevent the formation of molecular oxygen and hydrogen in overloaded lead accumulators, or to bind same gasiform oxygen and hydrogen. The bond may be effected by adsorption of the oxygen and hydrogen molecules, or formation of oxygen and hydrogen is prevented by chemical processes.

The invention further has the purpose to provide an accumulator which is able to work in every position whatever.

The solution of this problem proposed by the invention consists in creating a fluid and gas-tight totally-enclosed accumulator containing, besides electrolyte and electrodes, adsorbing substances as well as substances qualified to form a redox-process with the occurring gases.

It is required of these substances that they secure the slight reversibility of the redox-process. Moreover it is required of said substances that throughout the redox-process they do not substantially vary the potential differences in the accumulator.

Therefore such substances preferably are used which in initial condition as well as in reduced and oxidized state are insoluble in the electrolyte.

It is suitable to incorporate such substances into one or both electrodes or to add them on the electrodes. Substances of that kind do but trivially modify the potential differences and originate no noticeable self-discharge.

If the substances of the redox-system in initial condition are soluble in the electrolyte and at least partially dissociated, then they separate at the electrodes. Through this separation, however, the substances should not be allowed to form any compounds with the electrodes, or they should only form compounds difficultly soluble in the electrolyte. Besides, the reversibility should, of course, be assured.

Especially suitable for this purpose are polyvalent elements, for example oxides, acids and salts of chromium, titanium, vanadium, manganese, wolfram, molybdenum, uranium and the like. The properties which compounds out of said elements have in common are a good oxidizing and reducing effect.

Out of more, here are some compounds of said kind particularly suitable for acid accumulators, for example for lead accumulators:  $H_2Cr_2O_7$ ,  $CrO_3$ ;  $HVO_4$ ,  $V_2O_5$ ;  $H_2TiO_3$ ,  $TiSO_4$ ,  $H_2MoO_4$ ;  $H_2WO_4$ ;  $HMnO_4$ ;  $HReO_4$ .

These are thoroughly acids or oxides of the elements quoted. They have in common a tendency to forming complex compounds.

The property to form complex compounds deserves particular consideration why it generally implies still more favourable reducing effects. For this reason it may appear suitable not to add the customary compounds to the elements quoted, out of which the complex com-

2

pounds are formed afterwards, but to add primarily prepared concentrates of the complex compounds.

Following complex compounds may be mentioned for example to be applied in case of acid electrolytes: 5 Complex acids with silican or with a metal as central atom for example tetrachromic acid, metawolfram acid.

In case of basic electrolytes it will be more suitable, instead of acids or oxides, to use bases or salts of same elements or of similar ones.

10 Lead accumulators with sulfuric acid electrolytes form for example some heteropoly acids with the hydrogen separated at the cathode and with the oxygen separated at the anode and create in this way an effective redox-system. Periodic and vanadic acids should be mentioned as an example, for heteropoly acids. Further examples are heteropoly acids which are formed from vanadic acid with silicic acid, from vanadic acid with boric acid and from vanadic acid with telluric acid. Said heteropoly acids are added to the electrolyte.

20 Besides heteropoly acids, compounds of elements of the iron series are qualified to form a redox-system together with hydrogen and oxygen. In consideration of the easy but undesirable separation generally occurring at the electrodes when such compounds are used it 25 will be preferable to use compounds which are insoluble or at least nearly insoluble. Thus are said compounds substantially in suspension in the electrolytes. Examples thereof are basic sulfide of cobalt  $Co(OH)_S$  and of nickel  $Ni(OH)_S$ .

30 In a similar way titanium dioxide  $TiO_2$  or titanium (III) oxide  $Ti_2O_3$  form together with the oxygen and hydrogen separated at the electrodes an effective redox-system. Thereby the titanium dioxide or the titanium (III) oxide may be stored in the cathode for example 35 by mixing it up with the lead powder out of which the cathode is made by pressing method. Another means consists in spreading the titanium dioxide, respectively the titanium (III) oxide upon the surface of the cathode which in this manner is coated with a porous layer of

40 titanium dioxide, respectively of titanium (III) oxide. As a third possibility, the titanium dioxide, respectively titanium (III) oxide may be suspended in the electrolyte. In the latter case a larger quantity of titanium dioxide or titanium (III) oxide will be present than in the other cases where the substances are provided directly at or into the cathode.

45 In lead accumulators it is also possible to obtain effective redox-systems for realising the bond of gases occurring at the electrodes by incorporating iodine, arsenic, sulfur and chiefly selenium into the electrodes, preferably into the cathode, or by addition of same at the electrodes. An alternative possibility consists in solving iodic acid, telluric or tellurous acid, arsenic or arsenious acid, lead sulfide and preferably selenic acid or selenious acid in the 50 electrolyte.

As adsorbing substances it will be suitable to use such substances which have a very large surface and these may be suspended in the electrolyte. Most suitable for example is highly dispersed silicic acid which, when in suspension in the electrolyte, effects that the electrolyte 55 is converted into pasty state.

Although it is true that the bond of the gases is on the one hand already realised by the adsorbing substances and on the other hand by the substances forming a redox-system together with the gases separated at the electrodes, a practically useful effect is only attained through the co-operation of both kinds of substances.

60 In fact not only the gases themselves are adsorbed by the adsorbing substances, but equally the other substances of the redox-system. Latter thus are brought into a convenient position to react with the gases and, moreover, self-discharge is strongly reduced. Substantially the self-

discharge is conditioned by the diffusibility of the ions contained in the electrolyte. The diffusion, however, is strongly reduced by the adsorption and by the reduction of the ionic mobility as a consequence of the pasty consistency of the electrolyte.

In many cases, for example when the substances composing the redox-system are solved in the electrolyte and the accumulator is in overloaded condition, consequently when no self-discharge is menacing, a slight diffusion of the substances of the redox-system is desirable in view of good reaction conditions. Experiments have shown that it is possible to obtain a slight diffusion of the electrolyte in overloading state and a worse diffusion in resting state, by supplying the electrolyte in resting state with as great a quantity of adsorbing substances, for example highly dispersed silicic acid, as is necessary to make the electrolyte pass from the liquid state into a pasty consistency. By overloading and provided that the accumulator is gas-tight closed, the electrolyte spontaneously returns to liquid state as expected.

The invention is explained more in detail by means of following examples:

*Example 1*

In the sulfuric acid electrolyte of a lead accumulator—the concentration of the electrolyte has the value customary in lead accumulators—10 g. to 15 g. highly dispersed silicic acid having a surface of 300 m.<sup>2</sup> to 350 m.<sup>2</sup> per gram are suspended per 100 g. electrolyte.

In the negative electrode, titanium dioxide  $TiO_2$  is incorporated, namely substantially in that the titanium dioxide has been mixed up with the lead powder of the electrode and this mixture moulded to electrodes by pressing method. For a permanent loading current of 0.06 ampere, about 1.5 g. titanium dioxide  $TiO_2$  are sufficient.

In the course of the redox-process, by which the bond of oxygen formed at the anode and hydrogen formed at the cathode is realised, titanium (III) oxide is formed out of titanium dioxide and is re-converted into titanium dioxide. In view of the bond of the oxygen formed at the anode, this oxygen must be brought to the cathode. This can occur through diffusion, or in that the oxygen at first escapes and forms a gas-cushion above the electrolyte, and is solved in the electrolyte under the pressure of the gas-cushion. In the cathode, the bond is then realised of the oxygen by the titanium (III) oxide  $Ti_2O_3$  which was formed by reduction by the hydrogen formed at the cathode.

The voltage of this accumulator-cell during the loading process is of maximum 2.9 volts. The terminal voltage by beginning of the consumption of current is 2.2 volts.

Instead of pressing the titanium dioxide together with the lead of the cathode, titanium may be spread upon the surface of the cathode.

*Example 2*

Example 2 only differs from Example 1 in that the titanium dioxide  $TiO_2$  is not incorporated to the cathode nor spread upon its surface, but is suspended in the electrolyte. By same permanent loading current of 0.06 ampere a quantity of titanium dioxide  $TiO_2$  is, however, necessary which amounts to 2 to 3 g.

*Example 3*

Like in Example 1 silicic acid is added to the electrolyte of a lead accumulator. Further, as initial substance for the redox-process to realise the bond of oxygen and hydrogen, basic nickel sulfide  $Ni(OH)_2$  is suspended in the electrolyte. By permanent loading current of 0.06 ampere, 0.6 g. to 3 g. basic nickel sulfide are sufficient.

This accumulator-cell has a peak-tension of 2.6 volts during the loading process and a terminal voltage of 2 volts by discharge beginning.

The effect remains equivalent if, instead of basic nickel sulfide  $Ni(OH)_2$ , there is used basic cobalt sulfide

$Co(OH)_2$

5 About the same quantity is suspended in the electrolyte. Voltage conditions remain the same.

Equivalent effects also are obtained when basic nickel sulfide or basic cobalt sulfide, instead of being added to the electrolyte, are added to or embedded in the electrodes.

*Example 4*

Here again is a lead accumulator, to the electrolyte of which and in a like way as in Example 1 highly dispersed silicic acid has been added.

Besides this, the electrolyte contains a heteropoly acid formed from vanadic acid and per-iodic acid. The produced heteropoly acid, which is necessary for adding to an accumulator with a permanent loading current of 0.06 ampere, is formed from the reaction of 0.1 g. to 1 g. vanadic acid and an equal quantity of per-iodic acid in sulfuric acid of the concentration of an electrolyte of a lead accumulator.

Such an accumulator-cell has a peak-tension of 2.4 volts in course of the loading process and a terminal voltage of 2 volts by discharge beginning.

What I claim is:

1. A fluid and gas-tightly enclosed accumulator comprising, in combination, a fluid and gas-tightly closed casing; electrodes of opposite polarity arranged in said casing spaced from each other; an aqueous electrolyte located in said casing in contact with said electrodes, whereby during operation of said accumulator hydrogen and oxygen is generated; an adsorbent substance adapted to adsorb said thus generated hydrogen and oxygen, said adsorbent substance being insoluble in said electrolyte and dispersed in said electrolyte in finely subdivided state so as to at least retard accumulation of hydrogen and oxygen gas within said casing; and at least one oxidizable and reducible material selected from the group consisting of  $Ti_2O_3:TiO_2$  and of a heteropoly acid formed of substantially equal weights of vanadic and per-iodic acid, being located in said casing in contact with said electrolyte and present in a quantity sufficient to react with

30 substantially all of said hydrogen gas and oxygen gas generated during operation of said accumulator while said gases are at least partly adsorbed by said finely dispersed adsorbent substance, so as to prevent accumulation of hydrogen and oxygen gas within said casing.

35 2. An accumulator as defined in claim 1, said accumulator being of the lead-acid type and wherein said dispersed adsorbent substance consists of silicic acid.

40 3. An accumulator as defined in claim 1 wherein said oxidizable and reducible material is insoluble in said electrolyte forming a suspension therein.

45 4. An accumulator as defined in claim 2 wherein said oxidizable and reducible material is composed of  $Ti_2O_3:TiO_2$ .

50 5. An accumulator as defined in claim 2 wherein said oxidizable and reducible material is composed of a heteropoly acid formed of equal weights of vanadic and per-iodic acid.

55 6. An accumulator as defined in claim 2, wherein said oxidizable and reducible material is selected from the group consisting of  $Ti_2O_3:TiO_2$  being present in a quantity corresponding to between about 1.5 grams and 3 grams titanium dioxide at a permanent loading current of 0.06 ampere, and a heteropoly acid being present in a quantity equal to that formed from the reaction of between about 0.1 gram to 1 gram vanadic acid with a substantially equal quantity of per-iodic acid at a permanent loading current of 0.06 ampere; and wherein said silicic acid possesses a surface area of the magnitude of between about 300 and 350 square meters per gram, said silicic acid being present in a quantity equal to between

60 7. An accumulator as defined in claim 2, wherein said oxidizable and reducible material is composed of a heteropoly acid formed of equal weights of vanadic and per-iodic acid.

65 8. An accumulator as defined in claim 2, wherein said oxidizable and reducible material is selected from the group consisting of  $Ti_2O_3:TiO_2$  being present in a quantity corresponding to between about 1.5 grams and 3 grams titanium dioxide at a permanent loading current of 0.06 ampere, and a heteropoly acid being present in a quantity equal to that formed from the reaction of between about 0.1 gram to 1 gram vanadic acid with a substantially equal quantity of per-iodic acid at a permanent loading current of 0.06 ampere; and wherein said silicic acid possesses a surface area of the magnitude of between about 300 and 350 square meters per gram, said silicic acid being present in a quantity equal to between

about 10 and 15% of the weight of said aqueous electrolyte.

2,131,592  
2,631,115  
2,646,455

Lange et al. Sept. 27, 1938  
Fox Mar. 10, 1953  
Jeannin July 21, 1953

## References Cited in the file of this patent

## UNITED STATES PATENTS

5

|           |                 |               |         |
|-----------|-----------------|---------------|---------|
| 358,092   | Van Gestel      | Feb. 22, 1887 | 769,850 |
| 1,788,571 | Gardnier et al. | Jan. 13, 1931 | 166,707 |
|           |                 |               | 507,035 |

## FOREIGN PATENTS

|               |               |
|---------------|---------------|
| Great Britain | Mar. 13, 1957 |
| Great Britain | July 21, 1921 |
| Great Britain | June 8, 1938  |